

Jan. 19, 1954

C. C. HERITAGE

2,666,463

METHOD OF DENSIFYING WOOD

Filed Feb. 21, 1949



FIG. 1.



FIG. 2.

INVENTOR  
Clark C. Heritage

BY *Cook and Schermerhorn*

ATTORNEYS

## UNITED STATES PATENT OFFICE

2,666,463

## METHOD OF DENSIFYING WOOD

Clark C. Heritage, Cloquet, Minn., assignor to  
Weyerhaeuser Timber Company, Longview,  
Wash., a corporation of Washington

Application February 21, 1949, Serial No. 77,675

8 Claims. (Cl. 144—309)

1

This invention relates to the treatment of wood for the purpose of improving its structural properties and has particular reference to the permanent densification or compression of wood by the application of heat and pressure.

Various attempts have heretofore been made to compress both solid wood and wood laminated with cross banded sheets of veneer in order to improve the properties of the wood as a structural material; but the products of previously known processes have invariably had certain defects or shortcomings which seriously limited their utility and have prevented their general acceptance by the trade. In prior known treatments of wood for the purpose described the processes themselves have generally been quite restrictive in their applications. Some processes are considered to be applicable only to laminated veneers, or plywood, and not applicable to solid wood. Avoidance of a moisture content over a specified value has been recognized to be necessary, and the practice of preconditioning the wood to a relatively low moisture content has been generally adopted.

Attempts have also been made to increase the structural strength of the wood and to reduce its susceptibility to swelling and shrinking by treating the same with different chemicals prior to pressing of the wood. The present invention constitutes a signal improvement over such processes, inasmuch as it relies upon the utilization of only those substances contained in the wood in its natural state to achieve stable, permanent densification of wood.

According to prior art teachings the strength properties of the compressed wood do not seem to exceed values which would be expected of the original amount of wood substance. For example, the static bending and compressive strength properties ordinarily are increased by known processes in direct proportion to the increase in specific gravity. It is also taught that the wood retains its normal swelling tendency after compression so that if the volume is reduced to one-third of its original volume the swelling per unit of reduced volume is about trebled. This magnified swelling tendency and the general lack of permanence of the dimensions of the compressed wood in the presence of water constitutes one of the most serious and objectionable shortcomings of prior compressed wood products, notwithstanding claims for dimensional stabilization for certain products which are not borne out by experience. It is accordingly, a primary object of the present

2

invention to achieve substantial dimensional stabilization of wood which is permanent and effective, even in the presence of water.

Other important objects of the invention are to provide a densified wood having strength properties in excess of what would be expected of the wood merely on the basis of its increase in density; to provide a process for obtaining these improved properties without adding impregnating materials; to provide a process utilizing changes in substances found in natural green wood; and to provide a process applicable to green wood without preconditioning treatment. Still other and ancillary objects and advantages will become apparent in the following specification describing a preferred manner of carrying out the process.

The present invention involves the utilization of the original moisture in green wood to act as a natural plasticizer for thermosetting and thermoplastic substances in the wood, such as the native lignin, to cause these substances to act as a true plastic under conditions of heat and pressure. The invention contemplates the treatment of green wood, as the starting raw material, in two steps. In step I, the green wood, having a moisture content which may vary considerably but which is ordinarily about 70%, oven dry weight basis, is heated very rapidly and uniformly to reduce the moisture content to a value ranging from not less than 15% to the value represented by the fiber saturation point, which is ordinarily about 30% of the oven dry weight. The objective of step I is to reduce the original moisture content of the green wood to a value in the percentage range found practicable for the compression treatment of step II; and to do so with a minimum of alteration of the lignin as it occurs in its native state in order to obtain the maximum plasticizing and binding effect of the lignin in its highly reactive natural state. It is believed that the highly reactive natural state of the lignin is preserved, so long as the original moisture content of the green wood in the range of 70%, or higher, is maintained, but as the moisture drops below this value, the lignin is correspondingly altered, and the extent of alteration is proportional to the time the lignin is maintained at said reduced moisture content, either in direct proportion or possibly as a power function of the time. It will, accordingly, be appreciated that while it is necessary to reduce the moisture content to a value in the range satisfactory for compression treatment, such reduction should be made as quickly as possible,

not lower than the extent desired, and the sample should be subjected to the compression treatment of step II as quickly thereafter as possible and while the wood is still substantially at the maximum temperature developed in the moisture reducing treatment. In other words, the degradation of the lignin may be considered theoretically to be advanced in accordance with the product of (1) the time of exposure at, or association with, a moisture content reduced below that of the green wood, and (2) the extent of reduction of the moisture content below its normal "green wood" value. Since the moisture must necessarily be reduced to the range specified for the compression treatment, the only opportunity of capturing the native reactivity of the lignin with a minimum of degradation is to accomplish the moisture reduction process as quickly as possible and to no greater extent than necessary, and then to apply the pressure of the compression treatment in quick sequence. A third factor which undoubtedly influences the degradation of the native lignin is the subjection thereof to heat, particularly at reduced moisture content. It is accordingly desirable to avoid all excess heat in the moisture reduction step and to minimize the time of exposure to heat. However, since it is desirable, and facilitates the compression step, to apply the pressure under heat, it is accordingly advantageous to utilize all the heat absorbed by the wood in the moisture reducing step in order further to conserve time and reduce the total amount of heat absorbed.

In the second step of the process, which is conducted as quickly as possible after step I, as explained above, the wood is compressed under the influence of sufficient heat and pressure until its volume has been reduced to a fraction of its original volume, and then cooled while maintaining pressure. This step has for its objective the obvious result of increasing the density, and also to utilize the lignin, in the presence of the appropriate moisture content, as a combined plasticizer and resin to permanently bind the cellular tissues of the compressed fibrous material in its compressed condition to the maximum extent possible. It is believed that the lignin, or a wood substance generally regarded as lignin or as associated with the lignin, has thermoplastic properties and that the thermoplasticity is much improved by the presence of water. Whether for mechanical or chemical reasons, the optimum range of moisture content has been found by experience to be from about 15% to the fiber saturation point.

It is further believed that the lignin or a wood substance generally regarded and considered as lignin, also functions during this process step, somewhat in the manner of the condensation product of a thermosetting resin so that it first flows, and then cures, as the polymerization advances under the action of heat and the passing of time. The greater the extent to which this theoretical action of the lignin is accomplished, the more effective will be the resistance of the compressed wood to subsequent swelling or shrinking by water, and the more permanent will be its dimensional stabilization.

In the drawing, Figures 1 and 2 illustrate schematically the two steps of the process carried out in a hot press.

While it is ideally preferred to carry out both steps of the process in a continuous operation in a single machine, physical limitations of the apparatus, when using conventional presses, make

it expeditious to carry out the process in two distinct phases using a different apparatus for each step. The first of these phases of the process is identical with step I described above, and the second phase is identical with step II described above.

The process is typically illustrated in the treatment of a one-inch thick board of either flat or edge grain green wood having a moisture content far in excess of the fiber saturation value. The first phase of the process comprises the rapid heating of this green board in a high frequency dielectric field between metallic condenser plates to a uniform temperature slightly above 212° F. in order to reduce the moisture content to a value between 15% and the fiber saturation point in the shortest possible time. The moisture content at fiber saturation, of course, varies with the specific gravity of the wood, and the above value of 30% therefore represents the commonly accepted average value. The rate of heating is adjusted in accordance with the rate of moisture loss from the wood to produce the desired moisture content at the end of the first phase by the time the temperature reaches approximately 220° F., by controlling the electrical power output from a high frequency oscillator which is absorbed by the wood as a dielectric body. The driving off of the moisture is accompanied by formation of a cloud of steam, with the size of the cloud diminishing as the moisture content is reduced below the fiber saturation point.

The moisture content of the wood during the practice of step I may be conveniently determined by the variation in voltage across the condenser plate electrodes on opposite sides of the wood. Inasmuch as the power factor and capacitance decrease as the wood loses its moisture, the voltage across the plates for constant power input increases as the wood dries. Thus, by keeping the power input constant, the voltage readings may provide a direct indication of the moisture content. The fiber saturation point is very easily determined in this manner because of the electrical conductivity characteristics of wood containing free water in its grosser capillary structure. The electrical conductivity characteristics of wood do not vary as much with varying amounts of moisture content above the fiber saturation point, as they do in response to varying amounts of moisture content below the fiber saturation point. As completely or partially water filled wood is dried, the electrical conductivity changes rather slowly until the fiber saturation point is reached, the conductivity change for the entire range from completely water filled condition of the wood to fiber saturation point being only about 20 fold. As the wood dries from fiber saturation point, at about 30% moisture content to 7% moisture content, there is an approximately linear relationship between the moisture content and the logarithm of the electrical conductivity which produces a conductivity change over this range of over 100,000 fold. The break in the conductivity-moisture content relationship is thus so sharp that such variables as species, specific gravity of wood and variations in ash content, all have but slight effect on the conductivity in comparison with the effect of the moisture content. The rapid change in conductivity from 30% down to 7% moisture content also makes it relatively easy to determine the moisture content at any point in the range between 30% and 15% with which the present in-

vention is particularly concerned. The high frequency voltage between the electrodes may conveniently be measured by the use of a conventional vacuum tube voltmeter.

The temperature of the wood may easily be obtained by a thermo-couple embodied in one of the electrode plates wherein the plate may be of copper to form one of the thermo-couple elements. In such an arrangement, it is preferable to treat two pieces of wood at the same time on opposite sides above and below a center electrode containing the thermo-couple, whereby the thermo-couple is disposed at the point of maximum temperature of the assemblage to most effectively monitor the temperature to prevent charring of the wood. Outside electrodes above and below the top and bottom pieces of wood may then be connected together to the opposite side of a single output circuit, or individually to opposite sides of a push-pull circuit having its center wire connected with the center electrode. In either case, separate dielectric circuits are produced through the two pieces of wood. A simple dielectric circuit having two plate electrodes on opposite sides of a single piece of wood may also be used. Any temperature measuring device may be utilized, however, which operates satisfactorily under the conditions described. In all cases, the green wood should be insulated from the electrodes by the interposition of heavy fiber paper, thin dry wood veneer, or equivalent material to prevent short circuiting.

At the completion of the first phase of treatment, when the wood has attained a uniform temperature slightly above 212° F. and a moisture content of from 15% to 30%, it is immediately transferred to a hot press such as a conventional steam heated press having a platen temperature of 300° F. or higher. Side guards are provided to prevent the wood from spreading under pressure and thereby insure densification rather than mere displacement of volume. When using improvised platens, other pieces of green wood may be placed alongside the edges of the board determined by its lateral grain. Frictional resistance to displacement of said side guards under the pressure of the platens enables them to function as fixed abutments or side limits for the piece of wood being treated. In full scale commercial applications, spreading under pressure by the work may readily be prevented by using a closed mold. In the steam press a thin sheet of air dried veneer is preferably placed between the wood to be compressed and each of the hot platens to insure proper curing of the wood surfaces.

In a typical illustration of the process for the treatment of a one-inch flat grained Douglas fir board, there is preferably applied an initial pressure of about 800 pounds per square inch. This pressure is maintained for about 10 minutes, or until the parts of the wood remote from the platens attain a temperature above 320° F. At such time, the pressure is increased to 1400 pounds per square inch and held for 7 to 10 minutes. At the end of that time the wood is cooled to approximately room temperature in not less than 10 minutes while maintaining full pressure. After cooling, the pressure is reduced to atmospheric at a uniform rate in not less than 5 minutes; and then the wood may be removed from the press.

The above variables in the second phase of the process may be changed to accommodate different kinds and thickness of wood, 300° F. being

considered a lower limit of temperature for satisfactory stabilization and 375° F. being considered the maximum limit. The pressure necessary will, of course, depend upon the kind and density of the original wood and the temperature employed. For a given species of wood lower pressures may generally be used at higher temperatures, and higher pressures may be used with lower temperatures. A pressure in excess of 800 pounds per square inch is ordinarily necessary to produce compression of wood of near average density, a preferred pressure range for Douglas fir being between 1000 and 2000 pounds per square inch. Such pressures ordinarily produce a compression of the wood to about one-half its original thickness and volume. If greater densification is desired, higher pressures may be used.

Both phases of the process may be carried out in a press using high frequency heating exclusively, but certain factors make it desirable to heat the wood during the compression phase by thermal conduction from hot platens rather than by a high frequency field. While high frequency heating is ideally adapted to the rapid and uniform heating of the uncomplicated wood in the first phase, difficulties are incurred as the thickness of the wood diminishes under compression. If, for instance, a high energy output is applied to the dielectric field while wood having a high moisture content is under great pressure, explosions and disruptions of the wood are likely to occur. If the pressure is raised to relatively high values, as, for instance, above 7000 pounds per square inch while the wood is being heated in a dielectric field, the wood may become completely disrupted, the likelihood of disruption increasing as the wood dielectric becomes thinner. However, different woods respond differently, the danger being particularly great, for instance, in green hemlock and considerably less in Douglas fir.

Heating by high frequency current during the second or compression phase of the process also introduces the problem of maintaining perfect parallelism of the condenser plates. Any variation in the spacing of the plates results in uneven heating, which effect, of course, becomes greatly magnified as the plates more closely approach each other. Subject to such limitations as hereinabove pointed out, high frequency heating may be employed as the heating agency in the second or compression phase of the process as well as in the first phase.

To utilize the advantages of rapid dielectric heating in the first phase and hot platen heating in the compression phase, and, at the same time, avoid transferring the hot wood from the high frequency heater to the steam heated hot press between the first and second phases of the process, as hereinabove described, the high frequency heating circuit may be applied to the hot press itself which is then loaded in substantially cold condition. In such case the first step may be carried out under a relatively light pressure and without steam in the platens. After the rapid, uniform heating of the wood by the high frequency field to complete the first step, the electric power is turned off and the steam is turned on and pressure applied to the wood. During the second step all the heat is preferably then supplied by thermal conduction from the platens. To operate effectively, however, such a press should be specially designed to accommodate the condenser plates with proper provision for insulation and grounding; and with a special fa-

cility for quick heating of the platens by steam or electrical resistance to avoid loss of heat from the wood between the two steps of the process. In this procedure it is not necessary to handle the wood in hot condition; there is a minimum elapse of time between the completion of step I and the beginning of step II; and there is no potential across the plates to damage the wood while it is under high pressures.

Figures 1 and 2 illustrate how the two steps of the process may be carried out expediently in a single apparatus such as an electrically heated hot press, as described hereinabove. In Figure 1 light pressure is applied to the unheated platens and the wood is dried rapidly to the desired moisture content by the action of the high frequency heating circuit. Figure 2 illustrates the second step wherein heavy pressure is applied while the platens are heated by resistance elements in the platen heating circuit. The high frequency circuit is deenergized at this time.

Douglas fir boards compressed in the manner described above develop unexpected strength properties. As has been hereinabove mentioned, the strength properties of wood in general have heretofore been considered to be roughly proportional to the density of the wood regardless of the kind of wood. This principle has also been extended to apply to compressed wood treated according to prior art processes. However, using the process of the present invention, a green, flat-grained, Douglas fir board one inch thick having an original specific gravity of .59, when compressed to double its specific gravity, develops on the average a modulus of rupture in bending and a toughness by impact test of nearly two and one-half times the corresponding values of the original wood, and a compressive strength in a direction radial to the grain 16 times that of the original wood. The percent of swelling, as defined by change in thickness with respect to the original compressed thickness, for a number of samples, amounted to only 3 to 12% after 24 hours submersion in water. On the other hand, samples of Douglas fir boards compressed without regard to the critical conditions of the present process, to a specific gravity twice that of the original wood quickly swell to approximately the original thickness (90 to 100%) when immersed in water.

Douglas fir treated in accordance with the process of the invention is somewhat darkened, and its natural beauty is enhanced. When the compressed wood is sawed across the grain, the sawed end exhibits a fine, natural dark polish. Microscopic examination of a section perpendicular to the grain reveals that the spring wood is almost completely collapsed, the cells of the summer wood are partially collapsed, and the rays telescoped accordion fashion. The tendency to check and split is substantially reduced, and its wearing qualities, particularly for use as flooring material or the like, are greatly improved as indicated by the above comparisons with natural wood.

Western red cedar is more difficult to treat by the present process and its response to the treatment is not as uniform as that of Douglas fir, but does respond satisfactorily to the treatment with remarkable results. Cedar is lighter in weight and softer than Douglas fir and hence compresses more under the same conditions of pressure and temperature. For instance, under pressure and temperature conditions effective to reduce Douglas fir to about .4 of its original thickness, the cedar

is compressed to .2 of its original thickness. Good results have been produced with cedar compressed from an original specific gravity of .35 to a compressed specific gravity of 1.21, which is somewhat in excess of a 3.5 fold increase in density after allowing for the loss of moisture. Specimens have thus been produced having as low as 1% swelling defined by change in thickness after 24 hours submersion with respect to the original compressed thickness. The most remarkable improvement, however, is shown in the compressive strength in a radial direction with respect to the grain where strengths have been developed 45 times that of the original wood.

Since the specific gravity of wood substance itself is about 1.46, the exceptionally high strength properties developed by the present treatment cannot be accounted for merely on the basis of proportionality with respect to specific gravity according to the heretofore generally accepted rule. On this basis the strength properties of Douglas fir (original specific gravity —.59) could not be increased beyond an ultimate limit of about two and one-half times its original strength and Western red cedar could not be improved beyond four or five times its original strength, even if the wood were compressed to a solid condition with all the capillary spaces completely collapsed. It is, therefore, believed that the present process not only compresses the wood permanently to a denser condition with less energy than prior art processes, but also effects a marked change in the nature of the wood substance itself by the utilization of the plasticizing and the binding or resinous properties of the lignin or other reactive wood substances in the form nearest its original constitution or composition of its native state where its reactivity has been least altered, and it is this discovery that accounts for the greatly improved strength properties imparted to the wood, particularly in regard to its compressive strength.

The present process is particularly advantageous to increase the utilization of small pieces of wood which might otherwise be discarded as waste material or converted into material of less intrinsic value. Although wood thus treated is exceedingly hard and tough it may nevertheless be sawed and worked with the usual woodworking tools. When the surfaces are sanded they display a dark, almost lustrous finish, as though they had been stained and shellacked, making the wood particularly attractive as well as durable.

It is to be understood that the invention is not limited to the specific apparatus mentioned herein for carrying out the process, for various heating and pressing equipments may be devised by those skilled in the art to accomplish the general objectives stated in the specification. Neither is it intended that the invention be limited by the explanations of theory expressed herein should subsequent investigation show them to require alteration. It is to be further understood that various modifications of the process may be necessary in order to apply best the broad principles of the invention to different types of wood of different thicknesses and surface areas.

What is claimed is:

1. The method of treating green wood comprising rapidly heating the wood to reduce the moisture content to a predetermined amount in a range between 15% and the fiber saturation point and for plasticizing the native lignin in the presence of the remaining moisture, and immediately thereafter, before loss of a substantial

amount of the heat applied to the wood for reducing the moisture content, applying pressure to compress the wood to a predetermined thickness dimension.

2. The method of improving the structural properties of wood comprising rapidly heating green wood to reduce the moisture content thereof to a predetermined value within the range from 15% to the fiber saturation point for plasticizing the native thermoplastic and thermosetting substances in the wood in the quickest possible time in order to reduce to a minimum the degrading effects on said native thermoplastic and thermosetting substances of heat and time and existence in association with less than the moisture content of green wood, and immediately thereafter, with a minimum lapse of time and drop in temperature of the wood, applying pressure to the wood in hot condition to compress the same to a reduced volume, cooling the wood while maintaining the pressure to produce stable, permanent densification of the wood.

3. The method of improving the structural properties of wood comprising rapidly heating green wood to reduce the moisture content thereof to a predetermined value within the range from 15% to the fiber saturation point for plasticizing the native thermoplastic and thermosetting substances in the wood in the quickest possible time in order to reduce to a minimum the degrading effects on said native thermoplastic and thermosetting substances of heat and time and existence in association with less than the moisture content of green wood, and immediately thereafter, with a minimum lapse of time and drop in temperature of the wood, applying pressure to collapse and partially collapse the wood cells and to flow the native thermoplastic and thermosetting substances in the wood under the influence of the remaining original moisture content, cooling said wood to substantially room temperature while maintaining the pressure to set said substances and hold the wood cells permanently in said collapsed and partially collapsed condition and then removing said pressure.

4. The method of permanent densification of wood involving the utilization of a part of its original moisture content as a plasticizer for thermoplastic and thermosetting substances in the wood, comprising rapidly heating green wood uniformly throughout its mass to a temperature sufficiently high to plasticize native thermoplastic and thermosetting substances in the wood and to reduce the moisture content of the wood to a moisture content ranging from about 15% to the fiber saturation point, then immediately subjecting the heated wood to a pressure and temperature sufficient to compress the wood and flow said substances, and thereafter cooling the wood under pressure.

5. The method of improving the structural characteristics of wood comprising rapidly heat-

ing green wood to approximately 220° F. while retaining from 15% to 30% of the original moisture content of the wood, immediately subjecting said wood to a pressure of from 800 to 2000 pounds per square inch at a temperature of from 300° F. to 375° F., then reducing the wood to room temperature, and then removing said pressure.

6. The method of permanent densification of wood comprising rapidly heating green wood containing its original moisture in an alternating electrostatic field to a temperature slightly in excess of 212° F. and thereby reducing the moisture content to a value within the range of from 15% to fiber saturation, immediately subjecting the wood to pressure for a time sufficient to flow the native thermoplastic and therosetting substances in the wood, and then cooling the wood under pressure.

7. The method of permanent densification of wood comprising rapidly heating green wood containing its original moisture in an alternating electrostatic field to a temperature of approximately 220° F. and reducing the moisture content to a value in the range between 15% to 30%, immediately heating the wood to a temperature in the range between 300° F. and 375° F. and compressing the wood at a pressure in the range between 800 and 2000 pounds per square inch, and then cooling the wood under pressure.

8. The method of permanent densification of wood comprising rapidly heating green wood containing its original moisture in an alternating electrostatic field to a temperature slightly above 212° F. while reducing the moisture content to a value in the range between 15% and 30% at atmospheric pressure, then heating the wood to a temperature in the range between 300° F. and 375° F. and compressing the wood at pressures of from 800 pounds to 2000 pounds per square inch for approximately 14 to 20 minutes, then cooling the wood under pressure to approximately room temperature, and thereafter reducing the pressure to atmosphere in not less than five minutes.

CLARK C. HERITAGE.

References Cited in the file of this patent

UNITED STATES PATENTS

| Number    | Name      | Date          |
|-----------|-----------|---------------|
| 77,777    | Spaulding | May 12, 1868  |
| 1,952,664 | Esselen   | Mar. 27, 1934 |
| 2,089,644 | Samsonow  | Aug. 10, 1937 |
| 2,108,920 | Humiston  | Feb. 22, 1938 |
| 2,231,457 | Stephen   | Feb. 11, 1941 |
| 2,304,958 | Rouy      | Dec. 15, 1942 |
| 2,412,523 | Lundstrom | Dec. 10, 1946 |
| 2,529,862 | Bilhuber  | Nov. 14, 1950 |
| 2,543,618 | Wood      | Feb. 27, 1951 |

FOREIGN PATENTS

| Number | Country       | Date          |
|--------|---------------|---------------|
| 5,973  | Great Britain | Mar. 17, 1896 |